

1

3,582,257

**SOIL AND STAIN RESISTANCE AND SOIL AND STAIN RELEASE PROPERTIES IN TEXTILE ARTICLES**

Julian J. Hirshfeld and Bertie J. Reuben, Decatur, and John W. Bullington, Athens, Ala., assignors to Monsanto Company, St. Louis, Mo.

No Drawing. Filed May 10, 1968, Ser. No. 728,340  
Int. Cl. D06; D06m 9/00

U.S. Cl. 8—115.6

13 Claims

**ABSTRACT OF THE DISCLOSURE**

Textile articles of cellulosic fibers, of non-cellulosic fibers and comprising blends of cellulosic and non-cellulosic fibers, with improved soil and stain resistance qualities, and with minimized odor and toxicity in the finished product, are produced by contacting the articles with conventional press-free crease-retention thermosetting resin finish reactants containing an aldehyde or from which an aldehyde is released during polymerization thereof, animal glue, and a plasticizer; and by curing the resin.

**BACKGROUND OF THE INVENTION**

This invention relates to textile articles including fabrics consisting essentially of cellulosic fibers or of non-cellulosic fibers and fabric blends of both, and more particularly to a process for finishing textile articles including fabrics whereby soil and stain resistance and soil and stain release properties are enhanced.

Conventional "press-free," "wrinkle-free" or "permanent press" fabric finishing, as is known in the art, involves treating textile articles comprising cellulosic fibers, and preferably blends of cellulosic fibers and non-cellulosic fibers, with a resin. Although thermoplastic resins are sometimes used, this invention relates to the use of thermosetting materials in a process for imparting to a fabric or a garment the ability to retain its total shape-retaining properties indefinitely. When heated, these thermosetting materials react with a cellulosic substrate and/or with themselves to form insoluble, nonsoftening cross-links and resins in place. Many of the thermosetting materials contain formaldehyde or release formaldehyde when polymerized. This liberation of free aldehyde has presented a serious odor and toxicity problem with the use of such resin-forming materials as urea-formaldehyde monomers; ethyl, methyl and hydroxy ethyl carbamates; the triazones; the melamines; as well as the presently popular dimethylol, dihydroxy ethylene urea and dimethylol propylene urea. The relative desirability of the use of these resins has, in fact, been rated according to the amount of formaldehyde released.

As a general rule, fabrics finished with resins to create a permanent press are more easily soiled and have a tendency to resist stain removal, especially where the stains are of an oily or greasy nature. Fabrics which are blends of cellulosic fibers and non-cellulosic fibers are especially vulnerable to soiling and most resistant to soil and stain removal. This problem has been of great concern to dyers and finishers particularly as applied to white or light colored fabrics.

**SUMMARY OF THE DISCLOSURE**

It is a primary object of this invention to provide a process for improving soil and stain resistance and soil and stain release properties in textile articles, including fabrics consisting of cellulosic fibers, and/or non-cellulosic fibers,

2

It is a secondary object of this invention to provide for the removal by absorption of free formaldehyde released during the curing of certain thermosetting resins.

These and other objects and advantages will become apparent in the course of the following specification, examples and appended claims.

Briefly, the objects of this invention are accomplished in a press-free system by applying to the article a mixture of a thermosetting resin-forming material which contains formaldehyde or releases formaldehyde upon polymerization, a catalyst if required, animal glue or gelatin, and a plasticizer such as sorbitol or glycerine; and then curing the resin.

**DESCRIPTION OF THE PREFERRED EMBODIMENT**

The term textile article is meant to include fiber, yarn, all types of fabric, all types of carpets, and any textile article made of fiber. The textile article can be comprised of a natural fiber, a synthetic fiber or a combination of a natural and a synthetic fiber. Other types of material useful in textile articles and of common knowledge to the textile art may be present in minor portions. Examples of useful natural fibers include cotton, wool, silk, etc. The term synthetic fiber is meant to include all truly synthetic fibers and all man-made fibers. Examples of synthetic fibers include rayon fiber (a manufactured fiber composed of regenerated cellulose as well as manufactured fibers composed of regenerated cellulose in which substituents have replaced not more than 15% of the hydrogens of the hydroxyl groups), acetate fiber (a manufactured fiber in which the fiber-forming substance is cellulose acetate; where not less than 92% of the hydroxyl groups are acetylated, the term tri-acetate may be used as a generic description of the fiber), spandex fiber (a manufactured fiber in which the fiber-forming substance is any long-chain synthetic polymer of at least 85% by weight of a segmented polyurethane), polyester fiber (a manufactured fiber in which the fiber-forming substance is any long-chain synthetic polymer composed of at least 85% by weight of an ester of a dihydric alcohol and a dibasic acid or derivative thereof, such as terephthalic acid and dimethyl terephthalate), olefin fiber (a manufactured fiber in which the fiber-forming substance is any long-chain synthetic polymer composed of at least 85% by weight of ethylene, propylene or other olefin units), modacrylic fiber (a manufactured fiber in which the fiber-forming substance is any long-chain synthetic polymer composed of less than 85% but at least 35% by weight of acrylonitrile units), nylon fiber (a manufactured fiber in which the fiber-forming substance is any long-chain synthetic polymer having recurring amide groups as an integral part of the polymer chain), and acrylic fiber (a manufactured fiber in which the fiber-forming substance is any long-chain synthetic polymer composed of at least 85% by weight of acrylonitrile units).

The application of this invention is not restricted to a method of curing of the resin. Some of the resins mentioned herein are known in the art to be suitable for use in deferred curing processes; and some are known to be limited in use to pre-cured processes. Either process can be employed subject to material qualifications and limitations well known to those skilled in the textile art.

Not all resins and reactants which are used commercially to impart wrinkle-free properties to fabrics are suitable to the application of the instant invention.

Only those resins and reactants which contain aldehyde or in the curing process, release aldehyde to a greater or lesser extent, may be used without further addition of formalin or other aldehyde-releasing compounds. As used herein, unless otherwise indicated, the term "aldehyde-releasing resin" includes resin reactants containing

a free aldehyde as well as those forming an aldehyded when heat-cured. In either case free aldehyde is given off. The extent that free aldehyde is released during the curing process is, of course, determined by the particular resin reactants employed and by the conditions to which these reactants are subjected. Included within this group are the following:

(1) The urea-formaldehydes such as monomethylol urea



dimethylol urea



and trimethylol urea



which are produced from urea and formaldehyde, are used as reactants with formaldehyde, and release formaldehyde on curing.

(2) The melamine-formaldehydes including trimethylol melamine



hexamethylol melamine



and hexamethylol isomelamine



Like the urea-formaldehydes, the melamine-formaldehydes are normally produced in the presence of formal-

dehyde, the amount of formaldehyde controlling the degree of substitution in the condensing reaction. In the condensation to form resin, formaldehyde will be evolved with the use of each but considerably more will be evolved with the use of hexamethylol derivatives since there is no remaining N-hydrogen.

(3) The propylene ureas including dimethylol propylene urea



and dihydroxy dimethylol propylene urea



(4) The imidazolidones, made from urea and glyoxal, the most common of which used is dihydroxy dimethylol ethylene urea



(5) The carbamates including dimethylol ethyl carbamate



and dimethylol methyl carbamate



as well as dimethylol isopropyl carbamate



(6) The urons including dimethylol uron



and dimethyl N-methylol uron



## (7) The triazones including ethyl triazone



and

## (8) The acetals.

In connection with the use of the above finishing re-  
actants, it is only necessary that sufficient free aldehyde  
is released during the curing process to solidify the  
gelatin.

The techniques of employment of each is within the  
knowledge of those skilled in the art. We have found that  
with respect to these reactants, their use in quantities  
ordinarily employed in the art, will provide sufficient free  
aldehyde to solidify any useful amounts of animal glue.  
To provide a finish mixture in which substantially all  
formaldehyde is eliminated by absorption, it is necessary  
to determine the glue-resin ratio experimentally with re-  
spect to each resin. Where absorption of substantially all  
formaldehyde would require excessive amounts of glue,  
the elimination of odor by this method would, of course,  
be impractical.

The methylol resin-forming monomers require catalysts.  
Any suitable catalyst can be employed. Common among  
catalysts used in the polymerization of the above listed  
reactants are catalyst AC (trade name of the Monsanto  
Chemical Company for its approximately 50% solution of  
2-methyl 2-amino propanol hydrochloride), other amine  
hydrochlorides, organic acids, inorganic acids, ammonium  
salts, and certain metal salts (Lewis acids) such as zinc  
nitrate, calcium chloride and magnesium chloride.

Animal glue suitable for use in accordance with this in-  
vention is an impure gelatin obtained from animal organs  
by boiling with water, straining and drying, and is usually  
supplied commercially in thin, hard and brittle cakes. Vari-  
ous glue or gelatin materials of animal origin which are  
commercially available include acid-conditioned or lime-  
conditioned collagen from frozen pork skins and lime-  
conditioned collagen from calf skins, beef hides, and os-  
sein. The molecular weight of this natural polymer varies  
from about 20,000 up to about 250,000. Animal glue is  
essentially composed of polyamides of certain alpha-  
amino acids. It is believed that the amino acids are pres-  
ent not in the free state but rather as residues which are  
joined together by the elimination of water to form long  
polypeptide chains. Examples of some of the amino acids  
present in animal glue are glycine, proline, alanine, hy-  
droxyproline, glutamic acid, arginine, aspartic acid,  
leucine, valine, phenylalanine, isoleucine, meth-  
ionine, hydroxylysine, histidine, and tyrosine. Also it has  
been postulated that the animal glue molecules consist of  
single polypeptide chains terminated at one end by an  
amino group and at the other end by a carboxyl group.  
Description of useful animal glues can be found in Irvin  
Skeist, Handbook of Adhesives, 114-125 (1965); and in  
vol. 7, Kirk & Othmer, Encyclopedia of Chemical Tech-  
nology, 207-215 (1951).

Animal glue is generally an amber colored material  
which exhibits a crystal-like appearance in the dried  
ground form. Having no definite melting point, animal  
glue decomposes when heated to its charring tempera-  
ture. At temperatures of 100°-150° C., the glue exhibits  
a decreased solubility and an increased viscosity. Like most  
proteins, animal glue absorbs water readily and forms an  
elastic gel which readily melts at about 40°-50° C. to  
form a viscous solution having great adhesive properties.  
One of the characteristic properties of animal glue is its

tendency to form reversible gels in aqueous solutions.  
Such gels are characteristic of increasing rigidity with  
lower temperatures and rising concentrations. Gelatin of  
animal glue solutions can be prevented or retarded by  
5 the addition of inorganic soluble salts, e.g. salts of the  
alkali earth metals. Also, certain organic substances such  
as urea, thiourea and phenyl exhibit this liquefying power.  
Aqueous solutions of animal glue are quite stable over a  
10 wide range of pH values, e.g. 3.0-10.0, without appreci-  
able decomposition. The peptide units within the poly-  
mer of animal glue are subject to hydrolysis at tempera-  
15 tures above about 65° C. and boiling of an aqueous solu-  
tion of animal glue breaks down both the viscosity and  
jelly strength thereof and, in the presence of mineral acids  
or alkalies, such decomposition is almost instantaneous.  
An example of a useful animal glue is obtained by the  
hydrolysis of collagen:



wherein the chemical composition is:

|          | Percent |
|----------|---------|
| Carbon   | 51.29   |
| Hydrogen | 6.39    |
| Oxygen   | 24.13   |
| Nitrogen | 18.19   |
|          | 100.00  |

The use of the glue in accordance with this invention is  
not restricted to any particular source of gelatin material.  
Nor is the Bloom value of the glue of particular signifi-  
cance. It has been found that any amount of glue will  
improve soil resistance, but that amounts in excess of  
about 5% based on the weight of the fabric will impart  
a normally undesirable stiffness to the fabric.

The effect of formaldehyde on glue is well known in  
the glue arts. Even a trace, .4% or more, based on the  
weight of the glue, will solidify the glue into a substance  
which is insoluble in water. As the proportion of formal-  
dehyde to glue as the proportion of formaldehyde is in-  
creased; and as the proportion of formaldehyde exceeds  
about 50% the amount of the gelatin, there will be a  
marked deterioration in the soil resistance and soil re-  
lease properties of the finished fabric as the fabric is re-  
peatedly washed.

The amount of formaldehyde which will be absorbed  
45 by glue alone and which will provide maximum strength  
in the glue is within a range of 4-8%, based on the  
weight of the glue. This is the desirable amount of  
formaldehyde in the finish mixture when the fabric is  
50 comprised essentially of synthetic fibers. As the per-  
centage of cellulosic fibers in a fiber blend is increased,  
however, the amount of formaldehyde which reacts with  
cellulose should be added to the amount absorbed by  
55 the glue in determining a theoretically ideal proportion.  
The amount of formaldehyde which will react with and  
cross link cellulose under resin-curing conditions is known  
to approximate 5.8% in the case of dry cellulose and  
from about .4% to about 1.5% in the case of swollen cel-  
lulose, these percentages being based on the weight of the  
cellulosic fiber.

60 Suitable plasticizers for the animal glue in accordance  
with the instant invention include all alcohols, but prefer-  
ably one of the polyhydroxy alcohols, as, for example,  
sorbitol or glycerine. The plasticizers have no effect on  
the soil resistance or soil release properties of the fabric.  
65 Their only purpose is to prevent the glue from unduly  
adversely effecting the hand of the fabric. Therefore,  
where a soft hand is unnecessary or undesirable, the  
plasticizer may be omitted entirely. For most purposes,  
it has been found that a minimum of about 20% of a  
70 polyhydroxy alcohol based on the weight of the glue will  
provide a good hand in most fabrics. An excess in the  
amount of the alcohol plasticizer will not create an un-  
satisfactory product; however no useful purpose is served  
75 by including a polyhydroxy alcohol in excess of about  
500% based on the weight of the glue.

According to this invention, the plasticizer is mixed with an aqueous solution of the animal glue, which mixture, is, in turn, added to the resin formulation, followed by which the article is contacted with the mixture and subsequently cured.

It may of course be desirable to add other agents to the finish mixture in order to impart particular results. The inclusion of a rust inhibitor may be desirable where treated fabrics are likely to contact metals. A plasticizer or softening agent may also be included as an optional ingredient in order to provide a more desirable "hand" or texture to the treated fabric. It has been found that the cationic softening agent hydroxyl alkyl glyoxalidine can be employed for this purpose. Softening agents are normally employed in amounts of from about 1 to about 15% based on the weight of the total composition.

Contacting the textile article with the finish mixture can be accomplished by immersion, padding, spraying, roll application and any other such process known in the textile art. The contacting should be for a sufficient time to completely wet and impregnate the article. For example a contact time within the range of from about 5 minutes to about 90 minutes will generally be adequate to wet the textile article. A contact time of about 30 minutes is ordinarily preferred. However, preferred contact time for padding is from a fraction of a second to two seconds.

Following impregnation with the described treating composition, the treated fabric is dried and heated to cause reaction of the resin formulation, in situ, and to cure the resinous finish. At the same time the formaldehyde which is inherent in the resin system, is released as a free aldehyde, all or some of which is absorbed by the animal glue, causing the concomitant solidification of the glue in its plasticized form. The drying and curing of a treated fabric may be accomplished in separate steps or in a single operation if preferred. When drying is carried out as a separate step it may be done either at normal ambient air temperatures or at elevated temperatures from about 200° F. to about 250° F., leaving a residual moisture content of 5-8%. Following the drying operation, whether it be accomplished at normal temperature or by heating, the dried impregnated textile is brought to a temperature within the range of from about 260° F. to 350° F. The higher the temperature, the shorter is the period of heat treatment. Thus, drying the impregnated textile for 20 minutes in an oven maintained at a temperature of about 210° F. followed by heating at a higher temperature, for example, 8 minutes at 290° F. or for 4 minutes for 320° F., is generally effective in obtaining the desired results. These specific time and temperature periods are merely illustrative of those that can be employed.

Although as stated above, the application of this invention is especially suited and most effective when used with cellulosic fibers because the principles of cellulose reactivity are involved in cross-linking the cellulose by means of its available hydroxyl groups which are reactive sites for the resin reactants, this process has an important significance in connection with the non-cellulosic or synthetic fibers in fabric blends, and even with respect to fabrics composed solely, or in part solely of synthetic fibers. Even with the absence of available hydroxyl groups on the synthetic fibers, the use of the animal glue with its tendency to adhere to any fiber, creates, on the part of the non-cellulosic fibers a durable finish coating.

Permanent press finishes are most effectively applied to fabric blends of cellulosic and non-cellulosic fibers because there is a significant strength loss on the part of cellulose when finished with the durable press finishers. Since this strength loss ranges from 40 to 50%, synthetic fibers of polyester, nylon or acrylics are commonly used to maintain within the finished product a strength that is sufficient for the prospective end use. Accordingly, a resin finish which has a lasting effect on non-cellulosic fibers, as well as cellulosic fibers, is particularly useful in this new field.

The following examples will serve to illustrate specific embodiments of this invention.

### Examples

5 Swatches of a broad-cloth fabric blend consisting of 65% dacron polyester and 35% cotton were contacted with the following finish mixtures by dipping the fabric followed by padding on a mangle to a 65% wet pick up.

10

| Example | Ingredient                                                 | Percent by weight of fabric |
|---------|------------------------------------------------------------|-----------------------------|
| 1       | 40% solids solution of dihydroxy dimethylol ethylene urea. | 25.0                        |
|         | 30% solids solution of zinc nitrate.....                   | 4.5                         |
|         | Moropol 700.....                                           | 2.0                         |
|         | Silkand 40.....                                            | 2.0                         |
| 20      | 30% solids solution of dihydroxy dimethylol ethylene urea. | 25.0                        |
|         | 30% solids solution of $\text{CaCl}_2$ .....               | 4.0                         |
|         | Moropol 700.....                                           | 2.0                         |
|         | Silkand 40.....                                            | 2.0                         |
| 25      | 40% solids solution of dihydroxy dimethylol ethylene urea. | 25.0                        |
|         | 30% solids solution of zinc nitrate.....                   | 4.5                         |
| 30      | 30% solids solution of dihydroxy dimethylol ethylene urea. | 25.0                        |
|         | 30% solids solution of magnesium chloride.....             | 4.0                         |
|         | Cirrasol PT.....                                           | 10.0                        |
|         | $\text{CaCl}_2$ .....                                      | 10.0                        |
| 35      | 30% solids solution of dihydroxy dimethylol ethylene urea. | 25.0                        |
|         | 30% solids solution of magnesium chloride.....             | 4.0                         |
|         | Cirrasol PT.....                                           | 10.0                        |
|         | $\text{CaCl}_2$ .....                                      | 10.0                        |
|         | FC-216.....                                                | 1.5                         |
| 40      | 30% solids solution of dihydroxy dimethylol ethylene urea. | 25.0                        |
|         | 30% solids solution of magnesium chloride.....             | 4.0                         |
|         | FC-216.....                                                | 2.0                         |
|         | Animal glue.....                                           | 5.0                         |
|         | Sorbitol.....                                              | 5.0                         |
| 45      | 30% solids solution of dihydroxy dimethylol ethylene urea. | 25.0                        |
|         | 30% solids solution of magnesium chloride.....             | 4.0                         |
|         | Animal glue.....                                           | 5.0                         |
|         | Sorbitol.....                                              | 5.0                         |
| 50      | 30% solids solution of dihydroxy dimethylol ethylene urea. | 25.0                        |
|         | 30% solids solution of magnesium chloride.....             | 4.0                         |
|         | Animal glue.....                                           | 5.0                         |
|         | Sorbitol.....                                              | 5.0                         |
|         | $\text{CaCl}_2$ .....                                      | 10.0                        |
| 10      | Unfinished control.....                                    |                             |

NOTE.—The above trade names are identified as follows:

FC-216 by 3M Company is a soil release additive containing a fluorocarbon compound of the same family as "Scotchgaurd" chemicals.

Cirrasol PT by Imperial Chemical Industries, Ltd. is a soil release additive containing a polyester/polyethylene glycol copolymer and other undisclosed additives.

Silkand 40 by Onyx Chemical Co. is a softener of undisclosed composition.

Moropol 700 is a softener based on low density polyethylene by Morotex Chemical Co.

65 The saturated swatches were, in each case, cured for 20 minutes in an oven maintained at a temperature of 210° F. followed by an additional 8 minutes at 290° F. Sample 10, an unfinished control sample, was subjected to the same curing process.

70 All samples were pre-scoured with .25 g./l. of commercially available "Fab" detergent containing no optical brightener. The scouring was at a temperature of 140-150° F. for a period of 15 minutes. Samples were then rinsed, dried, and allowed to condition at room temperature and humidity. Their original reflectance was then

75

read against a white background with a Photovolt Reflectance Meter (Model No. 610, Photovolt Corp., New York, N.Y.). These readings are as shown in Table 1 under "original."

Each sample was then placed in a liter screw-cap jar containing 100 millimeters of a soiling solution, and the jar was agitated for a period of 5 minutes to insure that the sample was thoroughly saturated and well exposed to the mixture.

The soiling solution was prepared in the following manner. A 100 gram mixture consisting of

|               | Percent |
|---------------|---------|
| Palmitic acid | 10      |
| Stearic acid  | 5       |
| Coconut oil   | 15      |
| Paraffin      | 10      |
| Spermacetic   | 15      |
| Olive oil     | 20      |
| Squalene      | 5       |
| Cholesterol   | 5       |
| Oleic acid    | 10      |
| Linoleic acid | 5       |

was heated to 130° F., after which was added

|                 | Grams |
|-----------------|-------|
| Oleic acid      | 4     |
| Triethanolamine | 8     |
| Airborne soil   | 4     |

The above was mixed thoroughly and added to an equal volume of water at 130° F. in a Waring blender. After being homogenized for 15 minutes, the mixture was diluted to a liter and homogenized for another 15 minutes.

The samples were then removed from the screw-cap jars and passed through squeeze rolls with pressure adjusted on the rolls to provide cotton broad-cloth (3.1 oz./sq. yd.) with a wet pick-up of 70-80%. All samples were then hung in a circulating air oven set at 180-185° F. for 10 minutes. After drying, all samples were washed in a Tergotometer (U.S. Testing Co.) at 130° F. for 10 minutes at a 30:1 liquor-to-fabric ratio using 1 gram per liter of "Tide," a detergent soap manufactured by Procter & Gamble. Samples were rinsed, dried and again measured for reflectance with the Photovolt Reflectance Meter. Results of the second sample readings are at Table 1 under "whiteness after Soiling and Washing."

TABLE 1

| Example No.    | Original whiteness | Whiteness after soiling and washing | Percent change |
|----------------|--------------------|-------------------------------------|----------------|
| 1              | 91.0               | 57.8                                | 40.0           |
| 2              | 88.4               | 49.1                                | 44.4           |
| 3              | 81.0               | 73.6                                | 9.1            |
| 4              | 88.2               | 73.1                                | 10.0           |
| 5              | 101.9              | 99.4                                | 2.4            |
| 6              | 105.8              | 96.8                                | 8.5            |
| 7 <sup>1</sup> | 98.4               | 85.6                                | 12.1           |
| 8 <sup>1</sup> | 96.9               | 80.0                                | 17.4           |
| 9 <sup>1</sup> | 101.1              | 81.3                                | 19.5           |
| 10             | 113.0              | 94.2                                | 15.7           |

<sup>1</sup> Contain animal glue.

Soil resistance, as shown in the "% change" column, must be compared with stain resistance. Although some control samples without animal glue showed excellent soil resistant properties, their stain resistance was poor as shown in Table 2.

The same 10 samples were stained with 2 drops of each of the following stains: motor oil, mustard, Crisco, "3-in-1" oil, and mineral oil. The stains were allowed to dry, after which the samples were washed as described above. After washing and drying, the darkest portions of the stains were compared with the gray scale for evaluating staining, as described in Section II of the 1965 Technical Manual of The American Association of The Textile Chemists and Colorists. The degree of staining of each sample is shown as follows:

TABLE 2

| Sample No.     | Staining class | Description           |
|----------------|----------------|-----------------------|
| 1              | 1              | Heavily stained.      |
| 2              | 1              | Do.                   |
| 3              | 1              | Do.                   |
| 4              | 1              | Do.                   |
| 5              | 2              | Considerably stained. |
| 6              | 2              | Do.                   |
| 7 <sup>1</sup> | 4              | Slightly stained.     |
| 8 <sup>1</sup> | 4              | Noticeably stained.   |
| 9 <sup>1</sup> | 3              | Do.                   |
| 10             | 1              | Heavily stained.      |

<sup>1</sup> Contained animal glue.

Any departure from the description herein that conforms to the present invention is intended to be included within the scope of the claims.

We claim:

1. A process for providing a soil resistant and soil release finish to a textile article comprising the steps of contacting said article with an aqueous mixture consisting essentially of

(1) a resin-forming reactant selected from the group consisting of methylol urea, methylol melamine, propylene urea, imidazolidone, methylol carbamate, methylol uron, triazone and acetal,

50 (2) animal glue, and

(3) a polyhydroxy alcohol

and then curing said resin.

2. The process of claim 1 wherein said article is a fabric.

3. The process of claim 1 wherein said article is a fabric consisting essentially of cellulosic fibers.

4. The process of claim 1 wherein said article is a blend of cellulosic fibers and non-cellulosic fibers.

5. The process of claim 1 wherein said article is a filament.

6. A process for providing a soil resistant and soil release finish to a textile article comprising the steps of contacting said article with an aqueous mixture consisting essentially of

(1) a resin forming reactant selected from the group consisting of methylol urea, methylol melamine, imidazolidone, and methylol uron,

(2) a curing catalyst for said reactant

(3) animal glue, and

(4) a polyhydroxy alcohol

and then curing said resin.

7. The process of claim 6 wherein said article is a fabric.

8. The process of claim 6 wherein said article is a fabric consisting essentially of cellulosic fibers.

9. The process of claim 6 wherein said article is a blend of cellulosic and non-cellulosic fibers.

10. The process of claim 6 wherein said article is a filament.

11. A soil resistant finished textile article produced by 5 the process of claim 1.

12. A soil resistant wrinkle-free finished fabric comprising cellulose fibers produced by the process of claim 1.

13. A soil-resistant wrinkle-free finished fabric comprising cellulosic fibers and synthetic fibers produced by the process of claim 1. 10

## UNITED STATES PATENTS

|           |        |          |       |         |
|-----------|--------|----------|-------|---------|
| 2,884,301 | 4/1959 | Beaumont | ----- | 8—116.2 |
| 3,147,065 | 9/1964 | Koshar   | ----- | 8—116.2 |
| 3,362,782 | 1/1968 | Domenick | ----- | 8—116.3 |

GEORGE F. LESMES, Primary Examiner

B. BETTIS, Assistant Examiner

U.S. CL. X.R.

8—115.7, 116.2, 116.3, 127.6; 260—6; 117—139.4